

## UNITED STATES PATENT OFFICE

2,437,412

LATENT IMAGE INTENSIFICATION WITH  
SULFUR DIOXIDE

Walter J. Weyerts and Charles W. Wiederhold,  
Rochester, N. Y., assignors to Eastman Kodak  
Company, Rochester, N. Y., a corporation of  
New Jersey

No Drawing. Application July 26, 1945, Serial  
No. 607,273. In Great Britain November 8,  
1944

5 Claims. (Cl. 95—6)

1

This invention relates to photography and particularly to a method of intensifying a photographic latent image.

In Simmons U. S. Patent 2,368,267, granted January 30, 1945, a method for intensifying latent images is described according to which an exposed silver halide emulsion layer is treated before development with sulfur dioxide gas and then removed from the source of sulfur dioxide gas and stored for a period of time prior to development. This method produces satisfactory intensification of the latent image and an effective increase in speed of the sensitive material. However, it generally required long treatment times. If the sensitive material was kept in the atmosphere of sulfur dioxide for a short time, it has to be stored for about two days in air to secure the desired increase in speed. On the other hand, if the material were treated with sulfur dioxide for a long period, the time of air storage could be shortened but the total time of treatment remained considerable.

It is therefore an object of the present invention to provide a method for latent image intensification of photographic silver halide materials which does not require a long treatment time between exposure and development of the material. A further object is to provide a method for increasing the emulsion sensitivity or speed of photographic materials by a simple and rapid post exposure treatment so that the sensitive materials may be used under light conditions which previously had been considered unsatisfactory. A still further object is to provide a rapid method for treating underexposed films such as motion picture films to permit their salvage and utilization to form a satisfactory image. Other objects will appear from the following description of our invention.

These objects are accomplished by bathing an exposed silver halide emulsion layer, prior to development in an aqueous solution of sulfurous acid or a material which gives sulfurous acid in solution such as sodium bisulfite or potassium meta-bisulfite.

According to our invention, films or plates containing photographic latent images are bathed for approximately one minute in an aqueous solution of sulfurous acid or a material which furnishes sulfurous acid in aqueous solution, such as sodium bisulfite,  $\text{NaHSO}_3$  or potassium meta-bisulfite  $\text{K}_2\text{S}_2\text{O}_5$ . Alkali metal salts of other oxygen acids of sulfur which produce sulfurous acid in solution may be used. The sulfurous acid bath should not contain photographic developing

2

agents or materials which act as anti-oxidants such as hydroquinone or iso-ascorbic acid. Such materials completely arrest any latent image intensification and should therefore be excluded from the sulfurous acid bath. The pH of the bath should be maintained below about pH 6. The intensification of the latent image increases with increase in pH of the sulfurous acid bath but with the pH values above about pH 6 fog increases rapidly with rise in pH.

After treatment in the sulfurous acid solution, the films or plates are removed from the solution and the excess liquid removed from their surfaces by aid of an air squeegee or by wiping with a suitable material. They are then placed where air is free to circulate around them, for 10 to 20 minutes or longer after which they are developed in the usual manner.

The storage of the material in air after treatment in the sulfurous acid solution is an essential feature of our process. We have found that 10 or 20 minutes is a sufficient length of time to hold the treated material in air, although a longer period of time does no harm. The temperature and humidity of the air should be maintained at a point where no undue softening of the swollen, unhardened emulsion takes place. Although free circulation of air around photographic material during the holding period is desirable to obtain the maximum increase in sensitivity, a rapid circulation of air gives only little improvement over that obtained by merely hanging up a treated film in a darkroom for the required time. However, a film which has been treated and then placed in a small closed container during the holding period gives less increase in speed.

Our invention will be further illustrated by reference to the following examples. In comparing the effect of treatment in sulfurous acid solutions of exposed gelatino silver halide emulsions, with a control, it was found desirable to bathe the control in distilled water for the same length of time the material being tested was bathed in the sulfurous acid solution. The reason for this is that merely bathing a film in water before development gives a slight increase in speed over the original when both are developed under the same conditions. For this reason the controls were bathed in distilled water and then were held under conditions similar to the treated film before development.

## Example 1

A high speed negative gelatino silver halide emulsion such as Kodak Plus X was exposed on a standard sensitometer, for example, Eastman

Type 2B sensitometer, and portions of the film were then bathed in distilled water, in a 1% aqueous solution of sodium bisulfite and in a 1% solution of potassium meta-bisulfite for 1 minute. Each of these films was then removed from the solution and was held in air in the darkroom for 10 minutes. It was then developed in a solution of the following composition:

|                                   | Grams |
|-----------------------------------|-------|
| Monomethyl-p-aminophenol sulphate | 2.0   |
| Hydroquinone                      | 5.0   |
| Sodium sulfite                    | 100.0 |
| Boric acid                        | 8.0   |
| Borax                             | 8.0   |
| Potassium bromide                 | .25   |
| Water to 1 liter                  |       |

The films were then fixed in the usual way and the values for speed, gamma and fog were determined. The emulsion speeds were read as 30/E at a density of 0.3 above base color plus fog where E is exposure in meter candle seconds. The following results were obtained.

|                                                                                                | 30/E Speed | Gamma | Density of base +fog |
|------------------------------------------------------------------------------------------------|------------|-------|----------------------|
| <b>Control:</b>                                                                                |            |       |                      |
| Bathed in dist. H <sub>2</sub> O for 1 minute, held 10 minutes in air                          | 2,550      | 0.94  | 0.27                 |
| Bathed in 1% NaHSO <sub>3</sub> for 1 minute, held in air for 10 minutes                       | 3,800      | 0.84  | 0.27                 |
| Bathed in 1% K <sub>2</sub> S <sub>2</sub> O <sub>8</sub> for 1 minute, held 10 minutes in air | 7,050      | 0.73  | 0.26                 |

#### Example 2

A film such as that described in Example 1 was exposed in the same way as in Example 1 and portions of the film were then bathed for one minute in distilled water and in 1%, 2%, 5% and 10% aqueous solution of potassium meta-bisulfite. The films were then removed from the solutions and stored in air for 10 minutes after which they were developed in the same manner as in Example 1. The values for speed, gamma and fog were then determined with the following results.

|                                                                                                     | 30/E Speed | Gamma | Density of base +fog |
|-----------------------------------------------------------------------------------------------------|------------|-------|----------------------|
| <b>Control:</b>                                                                                     |            |       |                      |
| Bathed in dist. H <sub>2</sub> O for 1 minute, held in air for 10 minutes                           | 3,200      | 0.95  | 0.28                 |
| Bathed in 1% K <sub>2</sub> S <sub>2</sub> O <sub>8</sub> for 1 minute, held in air for 10 minutes  | 4,550      | 0.83  | 0.30                 |
| Bathed in 2% K <sub>2</sub> S <sub>2</sub> O <sub>8</sub> for 1 minute, held in air for 10 minutes  | 5,850      | 0.73  | 0.31                 |
| Bathed in 5% K <sub>2</sub> S <sub>2</sub> O <sub>8</sub> for 1 minute, held in air for 10 minutes  | 6,120      | 0.76  | 0.32                 |
| Bathed in 10% K <sub>2</sub> S <sub>2</sub> O <sub>8</sub> for 1 minute, held in air for 10 minutes | 5,000      | 0.82  | 0.30                 |

It will be understood that the examples and modifications included herein are illustrative only and that our invention is to be taken as limited only by the scope of the appended claims.

What we claim is:

1. The method of increasing the sensitivity of a gelatino-silver halide emulsion layer, which comprises exposing said layer to an actinic light image, immersing the undeveloped layer in an aqueous solution of an alkali metal salt of an oxygen acid of sulfur which produces sulfurous acid in solution, said first-mentioned solution

having a pH below about 6 and being free of photographic developing agent and other anti-oxidant, removing the layer from the solution and storing it in air for an appreciable period of time and then developing an image in said layer.

2. The method of increasing the sensitivity of a gelatino-silver halide emulsion layer which comprises exposing said layer to an actinic light image, immersing the undeveloped layer in an aqueous solution of sodium bisulfite having a pH below about 6 and free of photographic developing agent and other anti-oxidants, removing the layer from the solution and storing it in air for an appreciable period of time and then developing an image in said layer.

3. The method of increasing the sensitivity of a gelatino-silver halide emulsion layer which comprises exposing said layer to an actinic light image, immersing the undeveloped layer in an aqueous solution of potassium meta-bisulfite having a pH below about 6 and free of photographic developing agent and other anti-oxidants, removing the layer from the solution and storing it in air for an appreciable period of time and then developing an image in said layer.

4. The method of increasing the sensitivity of a gelatino-silver halide emulsion layer which comprises exposing said layer to an actinic light image, immersing the undeveloped layer in a 1% solution of sodium bisulfite having a pH below about 6 and free of photographic developing agent and other anti-oxidants, removing the layer from solution and storing it in air for approximately 10-20 minutes and then developing an image in said layer.

5. The method of increasing the sensitivity of a gelatino-silver halide emulsion layer which comprises exposing said layer to an actinic light image, immersing the undeveloped layer in a 1% solution of potassium meta-bisulfite having a pH below about 6 and free of photographic developing agent and other anti-oxidants, removing the layer from solution and storing it in air for approximately 10-20 minutes and then developing an image in said layer.

WALTER J. WEYERTS.  
CHARLES W. WIEDERHOLD.

#### REFERENCES CITED

50 The following references are of record in the file of this patent:

#### UNITED STATES PATENTS

| Number    | Name          | Date           |
|-----------|---------------|----------------|
| 1,424,062 | Agnew et al.  | July 25, 1922  |
| 1,850,162 | Wandt         | Mar. 22, 1932  |
| 1,973,446 | Crabtree      | Sept. 11, 1934 |
| 2,146,802 | Dersch        | Feb. 14, 1939  |
| 2,154,395 | Fricke et al. | Apr. 18, 1939  |
| 2,201,591 | Moreno        | May 21, 1940   |
| 2,311,103 | Weyerts       | Feb. 16, 1943  |
| 2,368,267 | Simmons       | Jan. 30, 1945  |

#### OTHER REFERENCES

65 Wightman, "Intensification of the Latent Image," Journ. Franklin Inst. 203 February 1927, pages 261 to 287 (pages 279 to 281 cited). (Copy in S. L.)

70 Bullock, "Chemical Reactions of the Photographic Latent Image," Eastman Kodak Co., 1927 (pages 145 and 146 of interest). (Copy in Division 7.)